

# UNITED STATES PATENT OFFICE.

FREDERICK SUPF, OF NEW YORK, N. Y., ASSIGNOR TO THE ARABOL MANUFACTURING COMPANY, OF NEW YORK, N. Y., A CORPORATION OF NEW YORK.

## PROCESS OF LIQUEFYING ORGANIC COLLOIDS.

974,448.

Specification of Letters Patent.

Patented Nov. 1, 1910.

No Drawing.

Application filed June 27, 1908. Serial No. 440,681.

To all whom it may concern:

Be it known that I, FREDERICK SUPF, a subject of the Emperor of Germany, and a resident of New York, in the county of New York and State of New York, have invented certain new and useful Improvements in Processes of Liquefying Organic Colloids, of which the following is a specification.

My invention relates to a process of treating organic colloids; and it has for its object to prevent, at ordinary temperatures, the coagulation of organic colloids, such as gelatin, glue, agar-agar, casein, starch and commercial dextrin (containing unconverted 10 or partly converted starch). I attain this liquefying effect by treating the aforementioned colloids with solutions of the salts of organic sulfonic acids, especially the salts of the inexpensive naphthalenesulfonic acid; 15 or with the salts of derivatives of sulfonic acids, such as polysulfonic, amido sulfonic, oxysulfonic, amido-oxysulfonic acids, etc. Amido groups, generally speaking, have the tendency to increase the liquefying effect. 20 The application of this property is of great value in the arts, being particularly useful in the preparation of adhesives, finishes and sizes. In the case of gelatin and glue for example, a neutral, non-hygroscopic, almost 25 colorless and odorless product is obtained and which is liquid at ordinary temperatures, highly concentrated if desired, as fluid as fish glue, more adhesive than the latter and dries more quickly.

In carrying out my process, for example in preparing a liquid hide or bone glue, I dissolve the dry glue in a warm solution (about 65° C. to 70° C.) of one of the aforementioned salts such as sodium naphthalenesulfonate, the ingredients being mixed together and well stirred and in substantially the following proportions by weight, viz.—hide glue, 300 parts; sodium naphthalenesulfonate, 80 parts; water, 400 parts. The mixture 35 after cooling possesses and retains the aforementioned valuable properties. The concentration of the solution of the salts is proportioned to the desired concentration of the glue, and varies with the coagulating properties of the crude glue.

The fact that a far larger quantity of sodium naphthalenesulfonate can be incorporated in the glue solution without crystallizing than could be dissolved in the quantity of water used for liquefying the glue,

and some other chemical facts, support the theory of the formation of a new complex, colloidal compound between the glue and the salt. This product, without losing in adhesive strength, differs from the original 60 glue by remaining liquid in the cold state. When dried and granulated, this glue possesses the valuable property of readily dissolving in cold water, and even in diluted alcohol, and of staying liquid as before, 65 whereas ordinary dry glue only swells up in cold water, must be heated in order to be dissolved, and must be kept warm while being used to prevent the same from gelatinizing.

It is known that formaldehyde renders animal glue insoluble. Now, animal glue, dissolved in hot water, jellifies as soon as formaldehyde is added and loses its adhesive properties almost immediately. When liquefied as previously described, however, 1 to 5% of commercial formaldehyde may be added, and the glue will remain liquid and adhesive for one hour or more. If 25% of alcohol, acetone or similar reagents are 70 added before the addition of the formaldehyde, the jellifying point is considerably retarded, the glue remaining liquid from 3 to 8 hours. The incorporation of the formaldehyde thus provides a water-proof glue 75 which remains liquid for a sufficiently long time to make it applicable to every day work.

Agar-agar, another example of an organic colloidal substance which gelatinizes at ordinary temperatures in 1 or 2% solution, is completely liquefied when treated with a saturated solution of sodium naphthalenesulfonate in the proportion of one to forty. Casein may be dissolved, for example, in a 90 warm solution (about 55° C.) of the sodium naphthalenesulfonate in substantially the following proportion by weight, viz.—dry commercial casein, 4 parts; sodium naphthalenesulfonate, 2 parts; water, 10 parts, and 95 as much alkali as required to neutralize, in whole or in part, the acid contained in the casein. Casein treated in the same manner and with the same quantity of alkali, but without the addition of the salt solution, 100 forms after cooling a solid coagulating mass, a fact which corroborates the liquefying action of the salt. Starch treated with about an equal amount by weight of sodium naphthalenesulfonate and boiled up with a de- 105

70

75

80

85

90

95

100

105

110

sired quantity of water, acquires properties similar to starch which has been treated with caustic soda, and coagulation is prevented. Sodium naphthalenesulfonate acts 5 in the same manner upon commercial dex- trins, especially white pasty dextrins which contain unconverted or partly converted starch. Dextrin solutions, so treated, be- 10 come transparent, more viscid, more tacky and gain in adhesive power and gloss.

I claim:

1. The herein described process of preventing or hindering the coagulation of cer- 15 tain organic colloids at ordinary tempera- ture, consisting in treating the colloids with a solution of a suitable salt of an organic sulfonic acid.
2. The herein described process of preventing or hindering the coagulation of cer- 20 tain organic colloids at ordinary tempera- ture, consisting in treating the colloids with a solution of a suitable salt of a derivative of an organic sulfonic acid.
3. The herein described process of preventing or hindering the coagulation of cer- 25 tain organic colloids at ordinary tempera- ture, consisting in treating the colloids with sodium naphthalenesulfonate.
4. The herein described process of preventing or hindering the coagulation of glue 30 at ordinary temperature, consisting in treat- ing said glue with a suitable salt of an organic sulfonic acid.
5. The herein described process of preventing or hindering the coagulation of hide 35 glue at ordinary temperature, consisting in treating the said hide glue with sodium naphthalenesulfonate.
6. The herein described process of pre-

venting or hindering the coagulation of hide 40 glue at ordinary temperature, consisting in treating by weight—300 parts of hide glue with 80 parts of sodium naphthalenesulfo- nate dissolved in 400 parts of water.

7. The herein described process of pre- 45 venting or hindering the coagulation of glue at ordinary temperature and of rendering the same waterproof, consisting in first treating said glue with a suitable salt of an organic sulfonic acid, and then with a suit- 50 able aldehyde.

8. The herein described process of pre- 55 venting or hindering the coagulation of ani- mal glue at ordinary temperature and of rendering the same waterproof, consisting in first treating said glue with sodium naph- thalene sulfonate, and then with 1 to 5% of formaldehyde.

9. The herein described process of pre- 60 venting or hindering the coagulation of glue at ordinary temperature and of rendering the same waterproof, consisting in first treating said glue with a suitable salt of an organic sulfonic acid, then with about 25% of alcohol or the like, and finally with 1 to 65 5% of a suitable aldehyde.

10. A neutral animal glue, which when mixed with formaldehyde will remain liquid at ordinary temperatures for a period of from eight to three hours, and then upon 70 drying become insoluble in water.

Signed at New York, in the county of New York and State of New York this 25th day of June A. D. 1908.

FREDERICK SUPF.

Witnesses:

FREDERICK DITTLER,  
A. F. VOIGT.